

## UNITED STATES PATENT OFFICE.

JOHN WESLEY MARDEN, OF EAST ORANGE, AND JOHN EDWARD CONLEY, OF BLOOMFIELD, NEW JERSEY, ASSIGNEES TO WESTINGHOUSE LAMP COMPANY, A CORPORATION OF PENNSYLVANIA.

## ACTIVATION OF ELECTRON-EMISSION MATERIAL.

No Drawing.

Application filed February 21, 1923. Serial No. 620,485.

This invention relates to the activation of material for electron-emission purposes and more particularly to the activation of such material prior to introduction into an electron device.

An object of our invention is the preparation of refractory filamentary material with activating material incorporated therein during the course of manufacture.

Another object of our invention is the introduction of carbon into filamentary material in a more compact form than heretofore, for activation purposes.

A further object of our invention is the preparation of filamentary material containing the required amount of electron-emission material combined with carbon or mixed with a carbon compound, whereby the volume percentage of such admixed material may be reduced to facilitate the working of the filamentary material.

A still further object of our invention is the preparation of carbides of thorium, tungsten and the like, for activation or other purposes.

Other objects and advantages will become apparent upon reading the following description.

Various methods have been proposed for liberating free thorium on the surface of electron-emission material for increasing the electron-emissivity thereof.

In the copending application of R. E. Myers, Serial No. 578,470, filed July 29, 1922, activation of thoriated filaments, and assigned to the Westinghouse Lamp Company, there is disclosed a method of preparing thoriated filamentary material with its surface so modified that upon heating, as an electron-emitting cathode, in an electron device, free thorium is developed on the surface thereof.

Briefly, the process comprises passing a thoriated filament, while heated, through a hydrocarbon atmosphere, comprising such compounds as benzene vapor or illuminating gas, whereby the thoria in the filament is either reduced to thorium, changed to thorium carbide or a mixture comprising one or more of the following materials is formed in or on the filament:—thorium, thorium carbide and tungsten carbide.

The process described in said application is only applicable for adapting material in

filamentary form for activation after introduction into an electron device. In order to prepare metallic material adapted to be drawn to filamentary form and activated by heating, without further treatment, upon introduction to an electron device, carbon and thoria have been mixed with tungsten powder, which mixture was subsequently pressed, treated and drawn to filamentary form in accordance with usual practice.

The disadvantage in such a procedure lies in the fact that free carbon is relatively light and therefore occupies a relatively large volume in proportion to its weight. The introduction of more than a very small proportion of carbon in this manner makes it more difficult to work the tungsten to filamentary form, because the difficulty in working tungsten, where foreign materials are added, is largely dependent upon the volume percentage of such foreign materials rather than on the percentage by weight.

To obviate the above noted difficulty, we propose to prepare activated filamentary material by mixing with tungsten powder, instead of a mixture of thoria and free carbon, either thorium carbide alone, or a mixture of thorium carbide and thoria or other thorium compound. If thorium carbide is used instead of free carbon, the volume percentage to be added for introducing the same weight of material is very much less than with free carbon. The volume percentage of thorium carbide necessary would be about  $\frac{1}{6}$  that of free carbon.

As an alternative, the mixture of thorium carbide and thoria may be used, in which case, they may be simply mixed with tungsten powder, pressed into a bar or slug, sintered either by the ordinary method in hydrogen or in a vacuum, if desired. Thorium carbide may be conveniently prepared by heating the metal powder to about 900° C. in an atmosphere of illuminating gas, benzene vapor or other hydrocarbon. For example, thorium carbide was prepared by heating thorium powder to about 900° C. for from two to three hours in a slow stream of illuminating gas, which was previously dried by passing through concentrated sulphuric acid.

Thorium carbide, alone, may be mixed with tungsten powder, the mixture pressed, treated and worked to the desired filamentary form.

tary form. In this instance, there will probably be enough oxide in the tungsten or enough oxidation introduced during the treatment, to at least partially decompose the thorium carbide to cause activation of the material. On the other hand, it is not necessary to have any free thorium present on completing the working of the wire. If all of the thorium is then in the form of thorium carbide, it may be desirable to have it that way, because of its greater stability than free thorium.

When heated to a sufficiently high temperature after introduction as a hot cathode in an electron device, the thorium carbide will either dissociate directly with the liberation of thorium, or will react with oxides necessarily present with the liberation of thorium.

In the following detailed description our invention is disclosed for producing activated tungsten but it is to be understood that we do not wish to be restricted to tungsten, for substantially the same method is applicable for producing activated molybdenum, tantalum and other similar refractory metals.

If it is desired to use thorium carbide alone for activating the tungsten, the same amount of carbide by weight may be used as is ordinarily employed for manufacturing thoriated tungsten, for example, 1 or 2% or less, by weight, may be admixed with tungsten powder. If a mixture of thorium carbide and thorium oxide or thoria are used, it is only necessary to employ about approximately half the quantity of the different ingredients.

The carbide or carbide and thoria are preferably very intimately mixed with tungsten powder, pressed into slugs of a convenient size, sintered or heat treated and finally swaged or rolled and drawn to the desired filamentary form. The same method of incorporating the carbide or carbide mixture may be used as is described and claimed in the copending application of W. B. Gero, Serial No. 618,396, filed February 10, 1923, manufacture of alloys or mixtures of metals and assigned to the Westinghouse Lamp Co., for incorporating thorium into tungsten, except that it is not necessary to use precautions to guard against oxidation of the carbide as it is for thorium. It should be appreciated that the only change from the custom-

ary method of preparing thoriated filamentary material, which is well known to those skilled in the art, is the addition of either thorium carbide alone, or admixed with thoria, instead of the usual proportion of thoria.

After drawing to the desired size of wire, the same may be introduced into an electron device, as the hot cathode thereof. Upon heating to incandescence, thorium will be developed or liberated in the filament, either by decomposition of thorium carbide, interaction between thorium carbide and thorium oxide, or between thorium carbide and tungsten oxide. Whatever the precise reaction or combination of reactions, good activation is produced because of the liberation or development of free thorium, at least on the surface of the filamentary cathode.

Although thorium has been disclosed as the preferred activating material, it is to be understood that our invention is applicable for activating by means of other electron-emitters such as uranium, zirconium and the like.

Although we have described what we now consider the preferred means of practicing our invention, it is to be understood that modifications will occur to those skilled in the art and we only wish to be restricted within the spirit and scope of the appended claims.

What is claimed is:

1. The method of manufacturing tungsten in filamentary form for electron-emission purposes comprising mixing with tungsten powder, a small proportion of thorium carbide, pressing said mixture to form a slug, heat-treating said slug and working to the desired filamentary form.

2. The method of manufacturing a refractory metal filament for electron emission purposes comprising mixing with the refractory metal powder a small proportion of a carbide of a metal of good electron emissivity, agglomerating said mixture into a bar, heat treating said bar and working and drawing the same to the desired filamentary form.

In testimony whereof, we have hereunto subscribed our names this 19th day of February, 1923.

JOHN WESLEY MARDEN.  
JOHN EDWARD CONLEY.